

# UNITED STATES PATENT OFFICE.

DENNIS ALDRICH, OF ST. LOUIS, MISSOURI.

## IMPROVEMENT IN PREPARING HIDES.

Specification forming part of Letters Patent No. 27,338, dated March 6, 1860.

*To all whom it may concern:*

Be it known that I, DENNIS ALDRICH, of the city of St. Louis, in the county of St. Louis and State of Missouri, have invented a new and Improved Process of Softening Dry Flint Hides Preparatory to Tanning; and I do hereby declare that the following is a full, clear, and exact description of the same.

As a green hide becomes dry by evaporation of its liquids its flesh surface forms a hard, flinty scale, to relieve the hide of which it has been customary to submit it during the softening process to the mechanical action of falling stocks or frequent and hard hand manipulations, which have to some extent the detrimental effect of loosening the small bundles of fibers composing the structure of the hide.

The object of my invention is to soften hides which have arrived at the above-specified condition, known as "flint hides," and dissolve the flinty scale without injuring the texture of the hides; and to this end my invention consists in treating such hides successively with diluted acetic acid and a solution of carbonate of ammonia, substantially in the manner described, as follows:

I first soak the hides in clean water until they become limber, and then immerse them in acid liquor composed of one (1) part, by weight, of acetic acid and sixteen (16) parts

water, allowing them to remain in this liquor until the scale is perfectly dissolved, which is generally effected in from twenty-four (24) to thirty-six (36) hours. The hides having thus had their fibers swelled and extended require to have the acetic acid extracted, and for this purpose I place them in a bath composed of seventy (70) parts, by weight, of water and one (1) part of carbonate of ammonia, and the acid combining readily with the ammonia forms acetate of ammonia, which, being very soluble in water, is easily washed out by subsequent washing in clean water. The time necessary for the hides to remain in the ammoniacal solution will be from twenty-four (24) to forty-eight (48) hours. The hides after this preparation are soft, their fibers are relaxed, and they are in a perfectly natural pliant condition.

What I claim as my invention, and desire to secure by Letters Patent, is—

The treatment of hides successively with diluted acetic acid and a solution of carbonate of ammonia, substantially as and for the purpose herein specified.

DENNIS ALDRICH.

Witnesses:

JAMES COFF,  
WOODFORD W. McCAMANT.